

Patented July 28, 1925.

1,547,799

# UNITED STATES PATENT OFFICE.

BENJAMIN G. FORREST, OF MERCHANTVILLE BOROUGH, NEW JERSEY, ASSIGNOR OF ONE-THIRD TO A. ARTHUR JONES AND ONE-THIRD TO CLAUDE L. ROTH, BOTH OF PHILADELPHIA, PENNSYLVANIA.

## METHOD OF SMELTING MIXTURES CONTAINING MAGNETITE DIRECTLY INTO STEEL METALS.

No Drawing.

Application filed February 1, 1923. Serial No. 616,403.

To all whom it may concern:

Be it known that I, BENJAMIN G. FORREST, a citizen of the United States of America, residing in the borough of Merchantville, county of Camden, and State of New Jersey, have invented a Novel Method of Smelting Mixtures Containing Magnetite Directly into Steel Metals, of which the following is a specification.

Where in the specification and claims I use the term "steel metal," I mean to describe iron, or iron alloy produced in a liquid condition, practically free from slag and from graphitic carbon, and sufficiently refined to be either malleable when cast or capable of hardening greatly by sudden cooling, or both, according to the percentages of carbon in the respective products of the various mixtures referred to in the context. When I use the term "ore", I mean to describe not only a metallic compound found in nature but also any concentrate of such a compound made by any means except smelting. Wherever I use the word "magnetite", I wish to be understood as meaning any form of magnetic oxide of iron, including any mixture of ores containing same, commonly called "black sands", derived from alluvial, beach or glacial deposits irrespective of the association of oxides of other metals with such oxide of iron when found in nature or concentrated. Where I refer to the percentages of different materials in any mixture or elements in any charge or product, I mean percentages by weight unless I state otherwise. By the expression "serviceable furnace" I mean any kind of container, other than a mere crucible, suitable for smelting mixtures containing magnetite by means of heat applied directly to such mixtures, or generated therein, or both, which can be used in the manner hereinafter described.

My invention relates to the direct production of divers steel metals from various mixtures of magnetite with other suitable materials, by smelting such mixtures by the aid of manganese ores or oxides included in such materials.

The principal objects of my invention are to make it profitable to use magnetite wholly or partly in the place of pig iron, wrought

iron or scrap metal in making various kinds of steel and alloy steels and to use certain ores of other metals, instead of their respective ferro-alloys, in conjunction with magnetite in producing divers alloy steels, which objects are obtainable by the method of smelting magnetite and materials mixed therewith hereinafter described.

Hitherto the chief obstacle to the direct production of steel metals from ordinary ores has been the large amount of impurities contained therein and purer ores such as magnetite have been considered too refractory for ordinary use. Consequently it has been customary, in making steel metals, first to reduce iron, only partly purified, from the low grade ores which are commonly used and then to refine it by some separate process and to add to it, while molten, all other elements, including alloys, necessary for the formation of steel or alloy steel of the desired composition. Frequently magnetite has been used in conjunction with hematite to bring up the yield of blast furnaces or as an addition to pig iron to fix the composition of steel in open hearth furnaces.

However I have discovered that if sufficient manganese ore or oxide of manganese be first mixed, in a serviceable furnace or crucible, with a charge composed chiefly of magnetite and carbonaceous matter and containing no low grade ore except such as may be needed to introduce desired fluxing or alloying materials therein, so that the quantity of impurities present which have a strong affinity for iron is relatively small, the mixture can be smelted directly into steel metal with the application of less heat than would be required if such manganese ore or oxide were not initially present, without requiring the use of any previously smelted or wrought iron or scrap metal as part of any such mixture, but such use or the addition of one or more ferro-alloys or scrap steel to such charge, either when mixed or when molten, may be of advantage in some cases, especially when making alloy steel, and I do not consider any such use as any departure from my process.

Furthermore, repeated tests have convinced me that the initial and continual presence in the charge of manganese ore or

oxide accelerates the chemical reactions occurring during the smelting of magnetite and other suitable materials mixed therewith as aforesaid not only while the iron and metals other than manganese in such mixture are being reduced to a molten mass but also after such reduction is practically completed so that then any oxide of manganese remaining assists in oxidizing the carbon remaining in the bath until the carbon content thereof is approximately that desired in the steel metal being made, when the elimination of carbon may be checked by casting or removing the charge or otherwise causing the temperature thereof to fall rapidly until the carbon no longer reduces any manganese, all the manganese meanwhile reduced assisting to remove any undesired elements or compounds not previously removed, by fluxing same into the slag or gases in the same manner that it does when reduced from additions to molten metal in other processes.

My invention is practiced by first commingling, in convenient form, in any serviceable furnace or crucible, a charge chiefly comprising magnetite mixed with one or more substances containing elements, metallic or otherwise, needed or useful; in addition to the iron in such magnetite, for making any desired steel metal that can be made in a continuous operation at the temperatures attainable in the apparatus used, including always sufficient carbonaceous matter to reduce and to carburize to the desired extent the metals to be smelted and to produce the heat necessary for smelting them, to the extent that it is to be generated from fuel within such container, with only a slight excess of such carbonaceous matter beyond the amount required for all such purposes, calculated as closely as practicable, and some ore or oxide of manganese from which manganese can be reduced in quantity not less than two per-cent of that of other metals to be smelted, if such manganese be not otherwise present in such mixture, and also any suitable flux or fluxes capable of removing any silica or other impurities also contained in such charge but not desired therein or admissible in such steel metal and by then heating such charge in such container by the combustion of such fuel or other means to the temperatures required to reduce from such charge and to alloy the steel making elements therein, say about 1,600 deg. centigrade, which temperatures will be attained with less consumption of fuel or applied heat under such conditions than if such matter containing manganese were not present, on account of the exothermic heat of chemical reactions caused or accelerated by the oxides of such manganese, including the oxidation of carbon monoxide

by such oxides of manganese, and by allowing the action of the manganese oxides to continue until the carbon in excess of the amount desired in the molten mass is oxidized also, when the metal should be cast or removed from the container in a liquid condition, separately from the slag, the manner of removing the latter being substantially like that practiced in the ordinary processes for making steel with containers and apparatus similar to those used for applying my process in any instance. The oxidation of excess carbon will be hastened by any increase and retarded by a decrease of the temperature of the molten mass after reduction of the metals desired in the bath is completed.

The composition of the resulting product may be modified, if necessary or desirable, while molten, by the addition of one or more ferro-alloys thereto or by other means of obtaining definite proportions of constituents desired in a final product not obtainable by the initial smelting operation. Either the initial or modified product may be cast into ingots for further treatment or otherwise shaped for industrial use.

The carbonaceous matter, whether used only as a reducing and carburizing agent or also as a fuel, may be introduced in one or more forms, either solid, liquid or gaseous, and as needed, after sufficient is put in the initial mixture to commence the reducing action, and likewise the other materials may be added in successive charges so as to keep the furnace or other apparatus in constant operation as long as it remains in fit condition for continuous use provided that such additions do not make it impracticable, considering the nature of the apparatus used, to oxidize the carbon in the molten metal in excess of the desired carbon content previous to the casting or removal of such metal or immediately thereafter while molten.

To insure the attainment of uniform results by my method, the conditions under which it is applied should be made as favorable to its operation as possible. For instance, care should be taken to select the constituents of the charge so that the total mixture will not contain more than one per cent by weight of either sulphur or phosphorus as my method affords no better means of eliminating those impurities than ordinary smelting practice except to the extent that the manganese or oxides thereof present assists in removing them. As magnetite containing less than one per cent of either sulphur or phosphorus can be prepared or concentrated without smelting much cheaper than pig or wrought iron can be produced, the advantage of using such magnetite instead of pig or wrought iron for making steel metals by my process will be obvious.

As "black sands" containing magnetite usually are roasted or sintered in preparation for smelting, the sulphur therein is almost completely removed by such preliminary treatment, and some of the other impurities likewise.

My method may be practised by means of various types of apparatus in common use, including open hearth furnaces, but crucible and electric furnaces are more suitable than others for controlling the composition of the products of smelting operations and expose the metals less than other furnaces to the absorption of sulphur from fuel and therefore are preferable for applying my process. Moreover, when the charge contains an ore more refractory than magnetite, it may be necessary to use an electric furnace to obtain the temperature necessary for the reduction of such ore, even though manganese oxide be present, but in all cases the presence of manganese ore or oxide in the initial mixture serves to reduce the amount of external heat required to smelt it.

The proportion of the various ores or compounds to be employed will be readily determined according to the requirements of each case by those skilled in the art and will depend on the percentages of various elements present therein and reducible therefrom and the relative percentages desired, not exceeding the amounts feasible to incorporate, in the final product, and of avoiding any excess of impurities, especially any containing sulphur, phosphorus and silicon, beyond the amounts readily removable in the smelting operation, considering the nature of the apparatus and of the fluxes to be used, but it should be assumed and my investigations have indicated that my method will not be effective on a commercial scale unless the charge to be smelted initially contains enough ore or oxide of manganese to contain manganese in quantity not less than two per cent of the weight of other metal or metals to be reduced. Any manganese needed for alloying purposes may be introduced initially in like manner in addition to the amount specified as essential for applying my process but it must be understood that less than one-half of the quantity required in the initial charge for smelting purposes will be retained in the final product, because most of the manganese either in metallic or oxide form will combine with impurities present and go off in the slag or gases. The quantity of magnetite expedient to use will depend upon the relative purity of the principal metallic materials mixed with it. It will be profitable to smelt magnetite in either large or small proportions with pig-iron, wrought iron, scrap or other refined metals, separately or in various combinations but when any ore other than magnetite is to be smelted therewith the latter should be sufficient to supply

at least one-half as much metal as all the other ores in such mixture, so as to keep down the percentage of gangue.

If the charge contains more than twenty per cent, of gangue, including silica, the slag will be excessive and interfere with the purification of the metal and make it difficult to keep it free from slag when cast or removed. While the use of materials good enough for the intended purposes and the proper mixing thereof are necessary conditions for the economical operation of my process, the most essential is putting and keeping in the charge more ore or oxide of manganese than is required to satisfy the affinities of elements or compounds present other than iron or oxygen for manganese. However I have found it impossible by my method to obtain a steel product containing less than 0.2% of manganese unless special means are employed when the metal is molten to lower the manganese content which may also be done without any departure from my process.

I do not consider the use of an air blast or other oxidizing agents for any purpose at any stage of the operations any departure from my process although I have found it possible to dispense with same when using ore or oxide of manganese as stated, and thus to avoid unnecessary occlusion of oxygen and oxides in the products of my process.

My method is therefore distinguishable among other respects from those hitherto used in making steel from mixtures containing magnetite in that my product may be produced entirely without the aid of any ordinary blast-furnace, Bessemer converter, additions of other ore or scrap as practiced in the open-hearth processes or methods of previously purifying the materials used in the crucible process, or the hitherto practiced additions of ferro-manganese or ferro-silicon or recarbureizers in any form to the molten metal during the final stages of production.

Obviously, the nature of the flux or fluxes to be used will depend on the character of the ingredients of the charge and practical steel-makers will know what the conditions in any given case require. I have found that it is generally necessary to form basic slags to remove silica and excesses of sulphur and phosphorus and that it is usually expedient to avoid using any furnace or crucible with an acid lining.

If the ores used in any case are so mixed as to be self-fluxing, no other flux will be needed.

Any oxide of titanium mixed or associated with the magnetite in the charge, or added thereto, will operate as an efficient flux for silica and other impurities that would otherwise combine with part of the manganese present either in metallic or oxide form.

4  
Therefore by my process ores containing more than 3% of titanic acid may be utilized as an original source of iron in conjunction with magnetite for steel making without increasing the difficulties of smelting the materials used, if no appreciable amount of titanium is desired in the final product, but I have found it impossible to make any alloy steel containing more than 1% of titanium out of mixtures of titaniferous ores with magnetite at any temperature below 1700 deg. centigrade although at higher temperatures I have made such steel by my process.

15 Of course, in every case, in addition to any requirements for fuel, enough carbonaceous matter, whether in solid, liquid or gaseous form, must be used to supply carbon or carbon monoxide in the quantity required to reduce all the desired metals and other elements from their ores or compounds and to carburize the iron to the extent desired which amount can be calculated within reasonable limits in all cases. When the 25 amount of carbon required cannot be calculated closely, a small excess of carbon should be used and samples of the molten metal taken and tested to determine when the charge should be cast to obtain the desired product, or one approximating same.

If in any instance the metal becomes or remains too highly carburized, its decarburization can be hastened by additions merely of high grade magnetite practically free 35 from sulphur, phosphorus and silica without any departure from my process.

It will be manifest to those skilled in the art, after understanding my invention, that modifications and substitutions of equivalents may be made in the materials to be mixed with magnetite for making steel metals by my method, such as the use initially of manganeseiferous iron ore instead of a simple ore or oxide of manganese, without departing from the spirit or scope of my invention and that my invention is not to be limited to any particular kind of apparatus or mixture of materials except to the extent that enough magnetite, carbonaceous matter, (either solid, liquid or gaseous) within the limits indicated, ore or oxide containing manganese in quantity not less than the minimum specified as essential to keep ample oxides thereof in the charge and suitable fluxes be used, substantially in the manner described, in any appropriate form of apparatus wherein any mixture containing said materials may be melted.

Furthermore, in conjunction with the 60 steps already described, any means of expeditiously, accurately or economically controlling, changing or fixing the carbon contents or hardening constituents or any component of any steel metal actually produced by my method of smelting mixtures contain-

ing magnetite may be employed without departing from the profitable use of such magnetite when mixed with some ore or oxide of manganese and, in some cases, with other ores or metals also, rather than the 70 use of refined iron or refined iron and one or more ferro-alloys, as the chief material, in the production of any steel or alloy steels respectively and I do not mean to limit my invention to the use of my method only in 75 connection with the processes of steel-making herein described.

Having now described my invention, what I claim as new and desire to secure by Letters Patent is the following:— 80

1. The metallurgical method, which consists of commingling magnetite, carbonaceous matter, suitable fluxes and some ore or oxide of manganese and smelting the mixture directly into steel metal by means 85 of sufficient heat, carbon or carbon monoxide, and the aid of such manganese or oxides thereof and fluxes, substantially in the manner described.

2. The metallurgical method, which consists of commingling magnetite, carbonaceous matter, some ore or oxide of manganese, and other suitable materials, including fluxes, needed for making steel metal of any special composition and smelt- 90 ing the same directly into such steel metal by means of sufficient heat, carbon or carbon monoxide, and the aid of such manganese or oxides thereof and fluxes, substan- 95 tially in the manner described. 100

3. The method of making a steel metal of a desired and feasible composition, which comprises the proper mixing of enough suitable materials, including magnetite, from which molten iron, free carbon, (or 105 carbon monoxide), an oxide of manganese and any other element or elements useful in making such steel metal can be obtained in a single operation upon the application of sufficient heat to such mixture in a serviceable furnace or crucible and smelting such mixture therein by means of such heat, carbon or carbon monoxide, and the aid of such manganese or oxides thereof and suitable fluxes, substantially in the manner de- 110 scribed, and adding to the charge when molten any additional elements not initially present but required to make such steel metal or otherwise changing the composition of the product of such smelting opera- 115 tion to attain the desired composition. 120

4. The herein described method of smelting various mixtures of materials, includ- 125 ing magnetite, carbonaceous matter, suitable fluxes and some ore or oxide of manganese, by means of sufficient heat, carbon or carbon monoxide, and the aid of such manganese or oxides thereof and fluxes, directly into steel metals with compositions varying with the respective elements obtain- 130

able and retained from the materials used in such mixtures respectively.

5. The herein-described method of accelerating the chemical reactions of smelting any mixture of materials, including magnetite and matter containing carbon, suitable for making any steel metal, which consists in initially using as part of such mixture some substance from which, when heated, 10 enough oxides of manganese will be derived to increase the exothermic reactions commenced by the heat so applied sufficiently to make the heat of such reactions aid materially in the complete smelting of such mixture.

6. In the art of incorporating manganese into any steel metal, the step which consists, in first mixing some ore or oxide from which at least the amount of manganese desired in 20 such steel metal and an excess equivalent in weight to one per cent of such metal can be readily reduced, with enough magnetite, carbonaceous matter and other materials needed or useful for making such steel metal, including suitable fluxes, and then smelting such mixture by means of sufficient heat, carbon or carbon monoxide, and the aid of such manganese or oxides thereof and fluxes and keeping the product molten until, 30 by oxidation or otherwise, the manganese contents thereof is fixed at the percentage desired or changed to same, substantially in the manner described.

7. In the art of incorporating any element other than iron, carbon and manganese into any steel metal, the step which consists in first mixing some substance from

which such additional element can be readily reduced, with enough magnetite, carbonaceous matter, ore or oxide of manganese and other materials needed or useful for making such steel metal, including suitable fluxes, and then smelting such mixture by means of sufficient heat, carbon or carbon monoxide, and the aid of such manganese 40 or oxides thereof and fluxes and keeping the product molten until such additional element has been alloyed with the iron to the extent desired by fusion or the percentage of same in the product has been otherwise fixed, substantially in the manner described. 45

8. In the art of making steel metal containing any element or elements, in addition to carbon, alloyed with iron, the step 55 which comprises the combination of such element or elements with such iron or with such iron and carbon during the process of smelting such iron, or the chief part thereof, from magnetite or a mixture of materials including magnetite, by means of sufficient heat, carbon or carbon monoxide, and the aid of manganese or oxides thereof and suitable fluxes contained in the initial smelting charge, substantially in the manner described. 60

In testimony whereof, I have signed my name to this specification, in the presence of two subscribing witnesses.

BENJAMIN G. FORREST.

Witnesses:

JOSEPH L. STRIFE,  
MAHLON HUNSBERGER.